

April 6, 1954

L. G. LUNDSTED  
POLYOXYALKYLENE COMPOUNDS

2,674,619

Filed Oct. 19, 1953

3 Sheets-Sheet 1

FIG. 1



Lester G. Lundsted  
INVENTOR.

BY *Richard J. Kelly*  
Attorney

April 6, 1954

L. G. LUNDSTED

2,674,619

POLYOXYALKYLENE COMPOUNDS

Filed Oct. 19, 1953

3 Sheets-Sheet 2

FIG. 2



Lester G. Lundsted  
INVENTOR.

BY *Richard D. Kelly*  
Attorney

April 6, 1954

L. G. LUNDSTED  
POLYOXYALKYLENE COMPOUNDS

2,674,619

Filed Oct. 19, 1953

3 Sheets-Sheet 3

FIG. 3



Lester G. Lundsted  
INVENTOR.

BY *Richard J. Kelly*  
Attorney

## UNITED STATES PATENT OFFICE

2,674,619

## POLYOXYALKYLENE COMPOUNDS

Lester G. Lundsted, Grosse Ile, Mich., assignor to  
 Wyandotte Chemicals Corporation, Wyandotte,  
 Mich., a corporation of Michigan

Application October 19, 1953, Serial No. 386,945

18 Claims. (Cl. 260—485)

1

This invention relates to a group of novel polyoxyalkylene compounds which have outstanding detergent and surface active properties, and in which the hydrophobic element is a polyoxypropylene polymer having a molecular weight of at least 900. This application is a continuation-in-part of my copending application, Serial No. 316,984, filed October 27, 1952, which is a continuation-in-part of my earlier filed application Serial No. 153,946, filed April 4, 1950, both applications now abandoned.

The art of producing surface active agents is old and well-developed, and it is a well-recognized principle that all such compounds are relatively large molecules which contain both hydrophobic and hydrophilic elements. The essential hydrophobic element in the prior art surface active agents has always been a hydrocarbon radical, such as found in the long chain fatty acids and alcohols, or in the alkylaryl group of the popular alkylarylsulfonate type detergents. The hydrophilic element has frequently been a polyoxyethylene chain, such as found in nonylphenol-ethylene oxide condensation products.

A serious limitation of the prior art surface active agents is that the structure of any particular surface active agent is relatively fixed and it is difficult to modify it, either as to molecular weight or the relative proportion by weight of the hydrophilic to the hydrophobic element. To prepare fatty alcohol based surface active agents having varying hydrophobic element chain lengths, it is necessary to use as many different starting materials as there are variations desired. Among the difficulties inherent in using several starting materials are the storage and handling of many types of complex organic compounds, supply problems as to rare homologues, the different reaction conditions required in preparing the surface active agents, etc., so that it is not feasible to prepare surface active agents which differ from one another in small, uniform increments of hydrophobic element chain length. Similar difficulties are encountered in preparing petroleum based surface active agents which differ from each other only in small, finite increments of hydrophobic element chain length.

A further shortcoming of prior art nonionic surface active agents is that all the highly active compounds are liquids or pastes. While the physical form of a surface active agent does not effect its surface active properties, convenience in packaging, distribution and use makes a solid form highly desirable.

Several United States Patents, e. g. 2,213,447; 55 polymer of at least 900 molecular weight. The

2

2,454,434 and 2,454,542—545, teach the use of polyoxyalkylene chains in surface active agents, but in all such patents the polyoxyalkylene chain constitutes the hydrophilic element of the surface active compound. U. S. Patent No. 2,425,845 discloses heteric or mixed polyoxyalkylene glycols, such as those which are formed when a mixture of ethylene and propylene oxides is condensed with a monoalkylene glycol, but these compounds do not possess detergent properties. It has also been previously known to react a higher aliphatic, water-insoluble monohydric alcohol sequentially with propylene oxide and ethylene oxide (U. S. Patent No. 2,174,761). The molecular weight of the polyoxypropylene chain in such a compound, even at its maximum theoretical value, is well below the minimum polyoxypropylene polymer molecular weight which has been found necessary in order to achieve the excellent detergent properties which characterize the compounds of the present invention.

It is an object of this invention to prepare novel polyoxyalkylene compounds having outstanding detergent and surface active properties and in which the hydrophobic element is a polyoxypropylene polymer.

Another object of this invention is to provide novel polyoxyalkylene compounds having excellent detergent and surface active properties and in which the molecular weight of both the hydrophobic and the hydrophilic element can be simultaneously varied within wide limits.

A further object of this invention is to provide nonionic detergents of high activity in a solid form.

Other objects and advantages of this invention will become apparent from the following detailed description thereof when read in conjunction with the accompanying drawings, in which:

Fig. 1 is a graph showing the effect of the polyoxypropylene polymer molecular weight upon detergent properties in 140° F. water.

Fig. 2 is a graph showing the effect of the polyoxypropylene polymer molecular weight upon detergent properties in 90° F. water, and

Fig. 3 is a graph showing the effect of variation of polyoxyethylene content on detergent properties in 140° F. water.

## NATURE OF INVENTION

A new class of polyoxyalkylene compounds has been discovered which have outstanding detergent and surface active properties and in which the hydrophobic element is a polyoxypropylene

50

55

novel polyoxyalkylene compounds are prepared by first condensing propylene oxide with an organic compound containing a plurality of reactive hydrogen atoms to prepare a polyoxypropylene polymer of at least 900 molecular weight, and subsequently condensing ethylene oxide, or its equivalent, therewith. The compounds of this invention conform to the following generic formula:



where

$Y$  is the residue of an organic compound containing therein  $x$  active hydrogen atoms,  
 $n$  is an integer,  
 $x$  is an integer greater than 1.

The values of  $n$  and  $x$  are such that the molecular weight of the compound, exclusive of  $E$ , is at least 900, as determined by hydroxyl number.

$E$  is a polyoxyalkylene chain wherein the oxygen/carbon atom ratio is at least 0.5, and  $E$  constitutes 20-90%, by weight, of the compound.

The significance of each element of the above generic formula will be set forth in the subsequent sections of this patent.

#### STRUCTURE OF THE NOVEL POLYOXYALKYLENE COMPOUNDS

The polyoxypropylene polymer, which is an intermediate in the preparation of the compounds of this invention, has the following structure:



wherein  $Y$ ,  $n$  and  $x$  are defined as in Formula A above. As is set forth in detail in a subsequent section of this application,  $Y$  is the residue of any organic compound containing a plurality of active hydrogen atoms. In the simplest case, when  $Y$  is the residue of propylene glycol, the polyoxypropylene polymer is simply a polyoxypropylene glycol of at least 900 molecular weight. If  $Y$  is the residue of a dibasic organic acid, e. g. adipic acid, the polyoxypropylene polymer has the following structure:



wherein  $n$  is defined as in Formula A.

The preferred compounds of this invention are prepared by condensing ethylene oxide, in an amount constituting 20-90% of the resultant compound, with the polyoxypropylene polymer. Thus, these compounds have the following formula:



where  $Y$ ,  $n$  and  $x$  are defined as in Formula A and  $m$  has a value such that the oxyethylene groups constitute 20-90%, by weight, of the compound. When ethylene oxide is condensed with a polyoxypropylene glycol of at least 900 molecular weight, the resulting compounds have the following structure:



where  $m$  and  $n$  are defined as previously set forth. When ethylene oxide is condensed with a polyoxypropylene polymer that is derived by the condensation of propylene oxide with adipic acid,

the resulting compounds have the following structure:



10

with  $m$  and  $n$  being defined as previously described.

The hydrophilic portion of the novel polyoxyalkylene compounds may be supplied by other polyoxyalkylene chains in lieu of the polyoxyethylene chain set forth in Formula C. Any polyoxyalkylene chain may be used provided that the oxygen/carbon atom ratio contained therein is at least 0.5. For example, such hydrophilic polyoxyalkylene chain may be derived from butadiene dioxide, glycidol, etc. By letting the symbol  $E$  represent generically any such polyoxyalkylene chain, Formula C may be rewritten as Formula A by simply substituting  $E$  for  $(C_2H_4O)_m$ . Formula A represents the broad generic class of compounds to which the present invention relates.

#### PREPARATION OF THE NOVEL POLYOXYALKYLENE COMPOUNDS

The preparation of the surface active agents of this invention involves two steps:

1. The condensation of propylene oxide with a base compound containing a plurality of reactive hydrogen atoms to prepare a polyoxypropylene polymer of at least 900 molecular weight, and

2. The condensation of ethylene oxide, or its equivalent, with the polyoxypropylene polymer.

In the first step propylene oxide is condensed with the base compound containing the plurality of reactive hydrogen atoms to prepare the polyoxypropylene polymer, viz:



Hereinafter the base compound containing a plurality of reactive hydrogen atoms will be referred to simply as the "reactive hydrogen compound." Alternatively, if desired, the polyoxypropylene polymer may be prepared by reacting a polyoxypropylene glycol with the reactive hydrogen compound, by esterification, etherification, etc. depending upon the nature of the reactive hydrogen compound, viz:



In the second step of the preparation, the hydrophilic polyoxyalkylene chain is introduced into the molecule by condensing ethylene oxide, or its equivalent, with the polyoxypropylene polymer, viz:



As an alternative procedure the hydrophilic polyoxyalkylene chain may be introduced by etherifying the polyoxypropylene polymer with a polyoxyethylene glycol, or its equivalent.

In preparing the polyoxypropylene polymer, the condensation of propylene oxide with the reactive hydrogen compound is normally carried out at elevated temperatures and pressures in the presence of an alkaline catalyst such as sodium alkoxide, a quaternary ammonium base, or pref-

erably sodium hydroxide. Similarly, the condensation reaction may be carried out in the presence of acid catalysts as set forth in U. S. Patent No. 2,510,540.

Although the reaction may be carried out by simply heating a mixture of the reactants under pressure at a sufficiently high temperature, this procedure is not ordinarily used as the temperatures and pressures required are excessive and control of the reaction is difficult. For each mol of propylene oxide reacting, an estimated 25 kilogram-calories of heat is liberated which, in the presence of a large quantity of propylene oxide, may increase the temperature and reaction rate to such an extent that the reaction assumes an explosive nature.

The preferred method of carrying out the reaction is to add the propylene oxide to a stirred, heated mixture of the desired reactive hydrogen compound and alkaline catalyst in a sealed reaction vessel. By adding the propylene oxide to the reaction vessel at such a rate that it reacts as rapidly as added, an excess of propylene oxide is avoided and control of the reaction is simplified.

The temperature at which the reaction is run will depend upon the particular system in question and especially upon the catalyst concentration used. Generally, at higher catalyst concentrations the reaction can be run at lower temperatures and correspondingly lower pressures. The temperatures and pressures required for any given reaction will vary with the reactive hydrogen compound, and the type and concentration of catalyst used.

The condensation of ethylene oxide with the polyoxypropylene polymer is carried out in an analogous manner.

The preparation of the novel polyoxyalkylene compounds of the invention is illustrated by Example 1 below:

#### EXAMPLE 1.—PART A

In a one-liter 3-neck round bottom flask equipped with a mechanical stirrer, reflux condenser, thermometer and propylene oxide feed inlet, there were placed 57 grams (0.75 mol) of propylene glycol and 7.5 grams of anhydrous sodium hydroxide. The flask was purged with nitrogen to remove air and heated to 120° C. with stirring, and until the sodium hydroxide was dissolved. Then sufficient propylene oxide was introduced into the mixture as fast as it would react until the product possessed a calculated molecular weight of 2380. The product was cooled under nitrogen, the NaOH catalyst neutralized with sulfuric acid and the product filtered. The final product was a water-insoluble polyoxypropylene glycol having an average molecular weight of 1620 as determined by hydroxyl number or acetylation analytical test procedure.

#### EXAMPLE 1.—PART B

The foregoing polyoxypropylene glycol having an average 1620 molecular weight was placed in the same apparatus as described in Part A of this example, in the amount of 500 grams (0.308 mol), to which there was added 5 grams of anhydrous sodium hydroxide. One hundred and five grams of ethylene oxide was added at an average temperature of 120° C., using the same technique as employed in Part A. The amount of added ethylene oxide corresponded to 17.4% of the total weight of the polyoxypropylene glycol base plus the weight of added ethylene oxide.

It will be noted in Part A of the above example that the molecular weight, as determined by hydroxyl number, was appreciably lower than the calculated molecular weight. Throughout this application, unless otherwise specified, it will be understood that the molecular weight of the polyoxypropylene polymer was determined by hydroxyl number using the method of Ogg et al., Industrial and Engineering Chemistry, Analytical Ed., vol. 17, p. 395, 1945.

#### EVALUATION TEST FOR SURFACE ACTIVITY

The following test procedure was used to evaluate the surface active properties of the products of this invention:

##### Carbon soil removal test procedure

A standard soiled cotton fabric is first prepared as follows:

Bleached, unfinished Indian Head muslin (58 x 47, 4.7 oz. per sq. yd., manufactured by Textron, Inc.) is used without pretreatment after conditioning to equilibrium at 65% R. H. and 70° F. A continuous 10 1/2 inch wide strip of the muslin is soiled by passing through an emulsion of colloidal carbon black and water-soluble mineral oil. After thorough impregnation of the standard muslin in the carbon black and oil emulsion, the cloth is passed through a power-driven household-type wringer to squeeze out any residual aqueous dispersion, the wringer pressure being so adjusted as to leave in the cloth an amount of standard soil dispersion equal to 120±5% of the dry weight of the cloth. The soiled muslin is then passed through a brush arrangement which by means of its mechanical action on the cloth controls the removability characteristics of the soil. The soiled muslin or test cloth is then dried, first in festoon under atmospheric conditions and then in an electrically heated, forced draft oven. After drying, the cloth is aged for 4 to 6 days by hanging in an atmosphere of 65% R. H. at 70° F. after which it is cut into test swatches measuring 2.5 inches±1/2 inch by 3.5 inches±1/2 inch using a power driven guillotine paper cutter. Before actual use of the so-prepared standard soiled cloth, it is checked for conformance with acceptability limits by the following described carbon soil removal test in standard detergent solutions. The swatches are stored at 65% R. H. and 70° F. prior to use.

To evaluate the soil removal characteristics of synthetic detergent compositions, 0.25% by weight solutions or other desired concentrations of the composition to be tested are prepared in water and 100 ml. portions of such solution are added to each of 10 one-pint jars of a "Launder-Ometer" (type 12Q-EF-SPA, manufactured by Atlas Electric Devices Company) standard laundry test machine.

Fifteen 1/4" diameter stainless steel balls are placed in each jar, after which two pieces of the previously prepared standard soiled cloth are added to each of nine jars. In the tenth jar are placed two pieces of unsoiled but pretreated cloth and this latter jar serves as a blank for determining the turbidity of the detergent solution. The so-prepared jars, heated to a temperature of 140°±2° F. in a constant temperature bath are then placed in the "Launder-Ometer" and run for 10 minutes at a speed of 42±2 R. P. M. The jars are then removed from the test machines and replaced in the constant temperature bath. The contents of each jar to which the standard

soiled cloth has been added are poured through a coarse screen to separate the steel balls and the standard soiled cloth from the soil suspension which is collected in a large beaker. The composite suspension thus attained is mixed thoroughly and a sample placed in a 20 mm. light absorption cell. The light absorption of this composite solution, as well as the light absorption of the solution in the tenth or "blank" jar containing the unsoiled cloth test pieces is then measured (by "Lumetron Colorimeter"). By means of a calibration curve for the "Lumetron Colorimeter," such curve being constructed by obtaining light transmission readings of known quantities of carbon black dispersion added to distilled water, the carbon soil removal value sought (in mg. of carbon per liter of solution) is obtained by taking the difference between the converted values of the light transmission of the composite solution or suspension from the nine jars and of the light transmission of the suspension in the blank jar.

The carbon soil removal values are then reported as a percentage of that of a standard detergent solution used as a reference or control material; viz. by dividing the mg. of carbon removal value of the test material composition by the mg. of carbon removal value for the standard or control detergent solution which is determined concurrently in the same test run and on the same standard soiled test cloth, and multiplying by 100.

The standard detergent solution used throughout the tests reported herein was a 0.25% solution of sodium kerylbenzene-sulfonate in distilled water. The sodium kerylbenzenesulfonate was prepared by effecting a Friedel-Crafts condensation of a chlorinated petroleum hydrocarbon distillate (derived from a hydrocarbon distillate having 9-16 carbon atoms and boiling in the range of 150-300° C.) with benzene and thereafter sulfonating the kerylbenzene compound to form the kerylbenzenesulfonic acid, which was subsequently neutralized with caustic soda to form the water-soluble sodium kerylbenzenesulfonate. After the neutralization of the sulfonic acid, sufficient sodium sulfate was added so that the final product contained 40% sodium kerylbenzenesulfonate and 60% sodium sulfate.

#### EFFECT OF POLYOXYPROPYLENE POLYMER MOLECULAR WEIGHT ON SURFACE ACTIVE PROPERTIES

A fundamental feature of this invention resides in the discovery that a polyoxypropylene polymer is sufficiently hydrophobic at a critical minimum molecular weight to serve as the hydrophobic element of surface active agents. The effect and criticalness of the polyoxypropylene polymer molecular weight upon surface active properties is illustrated by Example 2.

#### EXAMPLE 2

Eight polyoxypropylene polymers were prepared by condensing propylene oxide with propylene glycol following the procedure of Example 1, Part A. The molecular weights of the polyoxypropylene polymers were varied over a wide range and an approximately standard or uniform quantity (viz: 44-48% of the total weight of the product), of ethylene oxide was added thereto. The procedure of adding the ethylene oxide was the same as that employed in Example 1, Part B. Each of the compounds was then evaluated for carbon soil removal value at 140° F. by the pro-

cedure previously set forth. The results are set forth as follows:

TABLE I

| Run # | Molecular Weight<br>Polyoxy-<br>propylene<br>Polymer | Polyoxy-<br>ethylene<br>Content,<br>Percent of<br>Compound | Detergency,<br>Carbon Soil<br>Removal<br>0.25% at 140°<br>F. |
|-------|------------------------------------------------------|------------------------------------------------------------|--------------------------------------------------------------|
| 1     | 550                                                  | 45                                                         | 84                                                           |
| 2     | 763                                                  | 45                                                         | 83                                                           |
| 3     | 926                                                  | 45                                                         | 131                                                          |
| 4     | 938                                                  | 45                                                         | 131                                                          |
| 5     | 1,050                                                | 47                                                         | 217                                                          |
| 6     | 1,140                                                | 47                                                         | 228                                                          |
| 7     | 1,211                                                | 48                                                         | 244                                                          |
| 8     | 2,310                                                | 44                                                         | 232                                                          |

The data of the above table are plotted in the attached Fig. 1. It is seen that at polyoxypropylene polymer molecular weights of below 900 the detergency of the compounds is low, but that at approximately 900 molecular weight there is an inflection in the curve and the carbon soil removal value reaches 100% of standard. Above 900 molecular weight the curve climbs very rapidly to the approximately 225% of standard value at approximately 1100 molecular weight and then levels off, but stays at these high values.

As noted in the above example, all polyoxyalkylene compounds in which the polyoxypropylene polymer has a molecular weight of at least 900 have good detergency at 140° F., which is a conventional temperature used in laundry operations. The products of this invention in which the polyoxypropylene polymer portion has a molecular weight in excess of 2000 are a preferred embodiment of the invention in that they have exceptionally high detergency in cold water, viz. 90° F. The effect of polyoxypropylene polymer molecular weight on cold water detergency is illustrated in the following example.

#### EXAMPLE 3

Five polyoxypropylene polymers of varying molecular weights were prepared by condensing propylene oxide with propylene glycol following the procedure of Example 1, Part A. Ethylene oxide was added to each of the polyoxypropylene polymers to prepare compounds having an approximately equivalent quantity of oxyethylene groups (viz: 44-51% of the total weight of the product). Each of the compounds was then evaluated for carbon soil removal value at the low temperature of 90° F. The results are set forth in Table II below:

TABLE II

| Run # | Molecular Weight<br>Polyoxy-<br>propylene<br>Polymer | Polyoxy-<br>ethylene<br>Content,<br>Percent of<br>Compound | Detergency,<br>Carbon Soil<br>Removal<br>0.25% at 90°<br>F. |
|-------|------------------------------------------------------|------------------------------------------------------------|-------------------------------------------------------------|
| 1     | 1,100                                                | 48                                                         | 101                                                         |
| 2     | 1,270                                                | 44                                                         | 112                                                         |
| 3     | 1,620                                                | 51                                                         | 121                                                         |
| 4     | 2,320                                                | 44                                                         | 210                                                         |
| 5     | 2,600                                                | 47                                                         | 197                                                         |

The attached Fig. 2 is based upon the data of the above table. It is seen that at below molecular weights of approximately 2000 the cold water detergency lies within the range of approximately 100-120% of standard, but that at approximately 2000 molecular weight there is an inflection in the curve and that at all values in excess thereof the very high cold water detergency of 200% of standard or more is obtained. These results are particularly significant in that they exceed

the values that are obtained with the highest quality soap in much hotter water. Of course, the advantages of obtaining high detergency in cold water are obvious.

#### EFFECT OF POLYOXYETHYLENE CONTENT ON SURFACE ACTIVE PROPERTIES

The polyoxyethylene groups must constitute approximately 20-90% of the novel polyoxyalkylene compounds if good detergent values are to be obtained. The criticalness of this range is established by the following example:

##### EXAMPLE 4

Varying quantities of ethylene oxide were added to 2 polyoxypropylene glycols of 1270 and 2310 molecular weight following the procedure of Example 1, Part B, to prepare compounds having widely varying oxyethylene contents. The resulting compounds were subjected to the carbon soil removal test previously set forth and the results are shown in the following table:

TABLE III

| Run # | Molecular Weight<br>Polyoxy-<br>propylene<br>Polymer | Polyoxy-<br>ethylene<br>Content,<br>Percent of<br>Compound | Detergency,<br>Carbon Soil<br>Removal<br>0.25% at 140°<br>F. |
|-------|------------------------------------------------------|------------------------------------------------------------|--------------------------------------------------------------|
| 1     | 1,270                                                | 17                                                         | 68                                                           |
| 2     | 1,270                                                | 28                                                         | 91                                                           |
| 3     | 1,270                                                | 38                                                         | 146                                                          |
| 4     | 1,270                                                | 44                                                         | 202                                                          |
| 5     | 1,270                                                | 52                                                         | 225                                                          |
| 6     | 1,270                                                | 68                                                         | 206                                                          |
| 7     | 1,270                                                | 80                                                         | 141                                                          |
| 8     | 2,320                                                | 28                                                         | 115                                                          |
| 9     | 2,320                                                | 37                                                         | 216                                                          |
| 10    | 2,320                                                | 44                                                         | 232                                                          |
| 11    | 2,320                                                | 52                                                         | 214                                                          |
| 12    | 2,320                                                | 67                                                         | 208                                                          |
| 13    | 2,320                                                | 80                                                         | 175                                                          |

When the above data are plotted in Fig. 3, "bell shaped" curves are obtained which define the area of good detergency. It will be seen that the area of 20-90% encompass the area of good detergency, and wherein the curves rather abruptly change slope from the bordering low detergency values at below 20%, and above 90%, oxyethylene content. The limits of approximately 40-70% oxyethylene content pin point the area of maximum detergency. Essentially the same limits apply when other hydrophilic polyoxyalkylene chains, such as those derived from butadiene dioxide, glycidol, etc. and other alkylene oxides wherein the oxygen/carbon atom ratio is at least 0.5, are contained in the novel polyoxyalkylene compounds.

#### EFFECT OF Y ON SURFACE ACTIVE PROPERTIES

As noted heretobefore, the polyoxypropylene is prepared by condensing propylene oxide with a base compound containing a plurality of reactive hydrogen atoms. The function of the base compound is to furnish reactive hydrogen atoms which initiate the polymerization of the propylene oxide and, since the base compound constitutes only a small proportion of the high molecular weight polyoxyalkylene compounds, it ordinarily does not have an influence on the properties thereof. In other words, the particular base compound employed in preparing the novel polyoxyalkylene compounds is not critical so long as it furnishes at least 2 reactive hydrogen atoms, and operable polyoxyalkylene compounds are obtained regardless of the particular base compound employed in the preparation of the polyoxypropylene polymer. Ordinarily it is

preferred to employ relative low molecular weight base compounds, e. g. less than 200.

The term reactive hydrogen atom is well-known and clearly understood by those skilled in the art. However, to remove any possible ambiguity in this regard, the term reactive hydrogen atom, as used herein and in the appended claims, includes any hydrogen atom fulfilling the following two conditions:

1. It is sufficiently labile to open the epoxide ring of 1,2 propylene oxide, and
2. It reacts with methyl magnesium iodide to liberate methane in the classical Zerewitinoff reaction (see Niederl and Niederl, *Micro-methods of Quantitative Organic Analysis*, p. 263, John Wiley and Sons, New York city, 1946).

The reactive hydrogen atoms which will fulfill the above two conditions are normally activated by being a member of a functional group containing an oxygen atom, e. g. a hydroxyl group, a phenol group, a carboxylic acid group; a basic nitrogen atom, e. g. an amine group, a hydrazine group, an imine group, an amide group, a guanidine group, a sulfonamide group, a urea group, a thiourea group; or a sulfur atom, e. g. a mercaptan, a thiophenol, a thiocarboxylic acid, hydrogen sulfide. Alternatively, certain hydrogen atoms may be activated by proximity to carbonyl groups such as those found in cyanoacetic esters, acetoacetic esters, malonic esters, as is well known in the art. Specific examples of base compounds which may be used in preparing the polyoxypropylene polymers include ethylene glycol, 1,3 butylene glycol, oxalic acid, glycolic acid, mono-, di-, and triethanolamine, butylamine, aniline, resorcinol, diethylmalonate, etc.

The equivalency of all such base compounds in initiating the condensation of propylene oxide to form the polyoxypropylene polymer is illustrated by the following example.

##### EXAMPLE 5

Propylene oxide was condensed with, respectively, acetamide, 1,5 pentanediol, glycerine, ethylene diamine, benzene sulfonamide and sucrose to form polyoxypropylene polymers having molecular weights in excess of 900. The general procedure employed was that of Example 1, Part A except for certain minor changes in technique which will be obvious to those skilled in the art. Ethylene oxide was then condensed with the resulting polyoxypropylene polymers to prepare detergent compounds which were evaluated by the method previously set forth. The structure of the resulting compounds and the detergent values thereof are set forth in the following table:

TABLE IV

| 60 | Base Compound (Y)       | Molecular Weight<br>Polyoxy-<br>propylene<br>Polymer | Polyoxy-<br>ethylene<br>Content,<br>Percent of<br>Compound | Detergency,<br>Carbon Soil<br>Removal<br>0.25% at<br>140° F. |
|----|-------------------------|------------------------------------------------------|------------------------------------------------------------|--------------------------------------------------------------|
| 65 | Acetamide.....          | 974                                                  | 36                                                         | 164                                                          |
|    | 1,5 Pentanediol.....    | 1,372                                                | 50                                                         | 256                                                          |
|    | Glycerine.....          | 2,060                                                | 48                                                         | 265                                                          |
|    | Sucrose.....            | 5,060                                                | 49                                                         | 200                                                          |
|    | Ethylene Diamine.....   | 1,850                                                | 50                                                         | 271                                                          |
|    | Benzenesulfonamide..... | 1,179                                                | 50                                                         | 273                                                          |

70 While any reactive hydrogen compound containing 2 or more reactive hydrogen atoms may be used in preparing the polyoxypropylene compounds herein disclosed and claimed, the polyoxyalkylene compounds derived from certain specific base compounds have unusual and un-

expected properties which constitute invention over the generic class of compounds herein disclosed and claimed. For example, when arylsulfonamides are employed as the base compound, the resulting polyoxyalkylene compounds have excellent detergency at polyoxypropylene polymer molecular weights of only 700. Such compounds are more specifically disclosed and claimed in my copending application, Serial No. 279,794, filed April 1, 1952, now abandoned. Similarly, compounds derived from base compounds containing at least one nitrogen atom and at least one reactive hydrogen atom attached to a nitrogen atom, e. g. ethylene diamine, have exceptionally good cold water detergency and lime soap dispersing powers. Such compounds are more specifically disclosed and claimed in my copending application, Serial No. 349,283, filed April 16, 1953.

#### CHARACTERISTICS AND APPLICATIONS OF THE NOVEL POLYOXYALKYLENE COMPOUNDS

The compounds of this invention, in addition to the previously described outstanding ability to remove soil from a textile fabric (i. e. detergency is measured by carbon soil removal values) also possess remarkable ability to retain the soil suspended in solution once it is removed. This latter ability is measured by the "whiteness retention" test, described as follows:

##### Whiteness retention test procedure

Bleached, unfinished, clean Indian Head muslin, county 58 x 47, weight 4.7 oz./sq. yd. (Nashua Manufacturing Company), is cut into swatches measuring 2 1/2" x 3 1/2". The light reflectance of each side of every swatch is measured by means of a "Hunter Multipurpose Reflectometer" equipped with a green filter, using a standard white backing with a reflectance of 68.8% behind the cloth swatch. The average of such values of each side of each test piece is calculated and recorded. A standard soil suspension is prepared by diluting 28.55 grams of an aqueous carbon dispersion containing 35% carbon ("Aqua Blak B," Binney and Smith Co.) to 1 liter in a volumetric flask of distilled water.

A 0.25% distilled water solution of the detergent compound to be tested is then made up by adding 2.5 grams of the compound to a small amount of distilled water in a 1 liter volumetric flask. The previously prepared soil suspension is shaken vigorously and 50 ml. then pipetted into the flask containing the detergent. Sufficient distilled water is then added to this flask to make up to the one-liter mark.

The resultant mixture of detergent and carbon soil suspension is pipetted in 100 ml. portions into each of 5 "Launder-Ometer" jars, each jar containing fifteen 1/4" stainless steel balls. The jars and contents are brought to a temperature of 140° ± 2° F. in a constant water bath, then placed in the "Launder-Ometer" and rotated for 5 minutes at 42 ± 2 R. P. M. The "Launder-Ometer" is thereafter stopped and without removing the jars from the machine, the lids are opened and two standard cloth swatches, prepared as previously described, are placed in each jar after soaking for exactly 1 minute in distilled water without subsequent draining. The lids are replaced on the jars and the latter are rotated for an additional 30 minutes in the "Launder-Ometer." The swatches are then removed and immediately rinsed by flowing 3 liters of distilled water continuously through a rinsing flask while

shaking, and for a period of 5 minutes. Immediately after rinsing, the swatches are removed from the rinsing flask and placed on flat clean paper towels. The swatches are pressed dry on a laundry press set at a temperature of 328°-338° F. After pressing, the reflectance of both sides of each swatch is again measured by the "Hunter Reflectometer" and the average reflectance of all swatches calculated and recorded. The whiteness retention value is then calculated as follows:

Per cent whiteness retention (W. R.) =

$$\frac{\text{ave. reflectance after soiling} \times 100}{\text{ave. reflectance before soiling}}$$

The whiteness retention values are reported herein as a percentage of that determined in the standard detergent solution described under the "Carbon soil removal test procedure;" viz. by dividing the percent whiteness retention determined in the test material by the percent whiteness retention determined in the standard control detergent solution which is determined concurrently in the same test run and on the same standard test cloth, and multiplying by 100.

The numerical values obtained with several representative compounds of this invention are set forth in the table below:

TABLE V

| Run # | Molecular Weight Polyoxy-propylene Polymer * | Polyoxy-ethylene Content, Percent of Compound | Whiteness Retention 0.25% at 140° F. |
|-------|----------------------------------------------|-----------------------------------------------|--------------------------------------|
| 1     | 1,050                                        | 47                                            | 325                                  |
| 2     | 1,130                                        | 51                                            | 343                                  |
| 3     | 1,210                                        | 49                                            | 325                                  |

\* Condensation product of propylene oxide and propylene glycol.

The compounds of the present invention also possess excellent wetting properties, which are illustrated by the following tabulated results obtained by the Drave's Sink Time method [Technical Manual and Year Book of the American Association of Textile Chemists and Colorists, 25, 143-145 (1949)] employing 0.1% solutions of the compounds at 60° C. and using a 3 gram hook:

TABLE VI

| Run # | Molecular Weight Polyoxy-propylene Polymer * | Polyoxy-ethylene Content, Percent of Compound | Drave's Sink Time 0.1% at 60° C. |
|-------|----------------------------------------------|-----------------------------------------------|----------------------------------|
| 1     | 1,270                                        | 38                                            | 37                               |
| 2     | 1,210                                        | 49                                            | 33                               |
| 3     | 1,620                                        | 51                                            | 29                               |
| 4     | 1,620                                        | 64                                            | 39                               |
| 5     | 2,320                                        | 52                                            | 53                               |

\* Condensation product of propylene oxide and propylene glycol.

Illustrative of the surface tension lowering by the compounds of this invention are the following results:

TABLE VII

| Run # | Molecular Weight Polyoxy-propylene Polymer * | Polyoxy-ethylene Content, Percent of Compound | Surface Tension 0.1% at 25° C., Dynes/cm. |
|-------|----------------------------------------------|-----------------------------------------------|-------------------------------------------|
| 1     | 1,270                                        | 44                                            | 35                                        |
| 2     | 1,620                                        | 81                                            | 37                                        |
| 3     | 2,320                                        | 37                                            | 34                                        |
| 4     | 2,600                                        | 47                                            | 35                                        |

\* Condensation product of propylene oxide and propylene glycol.

A desirable characteristic of the polyoxyalkylene compounds of this invention is that both the hydrophobic and the hydrophilic elements thereof can be varied over an extremely wide range of molecular weights. By merely changing the quantity of propylene oxide added to the reactive hydrogen compound it is possible to prepare a wide range of hydrophobic elements that differ from one another in small, finite increments of polyoxypropylene polymer molecular weight. Similarly, varying quantities of ethylene oxide can be added to any of the above-described hydrophobic elements to prepare surface active agents, which differ from each other only in small, finite increments of polyoxyethylene content. By proper selection of reaction conditions, it is possible to vary over a wide range: (1) the hydrophobic polyoxypropylene polymer molecular weight, (2) the hydrophilic polyoxyethylene content and (3) the hydrophobic polyoxypropylene polymer molecular weight/hydrophilic polyoxyethylene content ratio. The facility with which the structure of the surface active agents can be varied is highly advantageous in that surface active agents can be "tailor made" to perform specific functions.

In addition to their surface active properties, the polyoxyalkylene compounds of this invention have many other diverse applications in the industrial arts. For example, these compounds have an excellent plasticizing action on a wide range of thermoplastic and thermosetting resins. In this regard, attention is directed to the pending applications of Lester G. Lundsted and J. P. McMahon, Serial No. 231,656, filed June 14, 1951, and Serial No. 259,476, filed December 1, 1951.

In the appended claims, the term "cogeneric mixture" is used. This is a term that has been coined to designate a series of closely related, touching homologues that are obtained by condensing a plurality of alkylene oxide units with a reactive hydrogen compound (see United States Patent 2,549,438, particularly the section beginning at column 12, line 40).

Also in certain of the claims, organic compounds containing a plurality of reactive hydrogen atoms are defined as having a detergency factor of less than 100. The detergency factor is the measure of the detergent-forming, hydrophobic character of any organic compound containing one or more reactive hydrogens and is determined as follows:

Varying quantities of ethylene oxide are added to the reactive hydrogen compound to prepare oxyethylene adducts containing  $20 \pm 5\%$ ,  $30 \pm 5\%$ ,  $40 \pm 5\%$ ,  $50 \pm 5\%$  and  $60 \pm 5\%$  oxyethylene content. Distilled water solutions of 0.25% concentration are prepared with each of the adducts. The carbon soil removal value of each adduct is determined at  $140^{\circ}$  F. following the procedure described by Vaughn and Suter, The Journal of the American Oil Chemists' Society, vol. XXVII, No. 7, pp. 249-257. As a control, the carbon soil removal value of an 0.25% distilled water solution of a standard sodium alkylarylsulfonate detergent is determined concurrently at  $140^{\circ}$  F. and on the same batch of soiled cloth. The standard detergent is sodium kerylbenzenesulfonate which is prepared by effecting a Friedel-Crafts condensation of a chlorinated petroleum hydrocarbon distillate (derived from a hydrocarbon distillate having 9-16 carbon atoms and boiling in the range of  $150$ - $300^{\circ}$  C.) with benzene and thereafter sulfonating the kerylbenzene com-

pound to form the kerylbenzene sulfonic acid, which is subsequently neutralized with caustic soda to form the water-soluble sodium kerylbenzenesulfonate. After the neutralization of the sulfonic acid, sufficient sodium sulfate is added so that the final product contains 40% sodium kerylbenzenesulfonate and 60% sodium sulfate.

The carbon soil removal values of the oxyethylene adducts are reported on a comparative basis with the standard sodium alkylarylsulfonate detergent being assigned an arbitrary value of 100. The highest carbon soil removal value obtained with the five oxyethylene adducts is then taken as the detergency factor of the reactive hydrogen compound.

What is claimed is:

1. A cogeneric mixture of conjugated polyoxypropylene-polyoxyethylene compounds containing in their structure oxypropylene groups, oxyethylene groups and an organic radical derived from an organic compound containing a plurality of reactive hydrogen atoms; the compounds being characterized in that all of the oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 900, as determined by hydroxyl number, and the oxyethylene groups present constituting 20-90%, by weight, of the mixture.

2. A cogeneric mixture of conjugated polyoxypropylene-polyoxyethylene compounds containing in their structure oxypropylene groups, oxyethylene groups and an organic radical derived from an organic compound containing a plurality of reactive hydrogen atoms; the compounds being characterized in that all of the oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 900, as determined by hydroxyl number, and the oxyethylene groups present constituting 40-70%, by weight, of the mixture.

3. A cogeneric mixture of conjugated polyoxypropylene-polyoxyethylene compounds containing in their structure oxypropylene groups, oxyethylene groups and an organic radical derived from an organic compound containing a plurality of reactive hydrogen atoms; the compounds being characterized in that all of the oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 2000, as determined by hydroxyl number, and the oxyethylene groups present constituting 20-90%, by weight, of the mixture.

4. A cogeneric mixture of conjugated polyoxypropylene-polyoxyethylene compounds containing in their structure oxypropylene groups, oxyethylene groups and an organic radical derived from an organic compound containing a plurality

15

15  
of reactive hydrogen atoms; the compounds being characterized in that all of the oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 2000, as determined by hydroxyl number, and the oxyethylene groups present constituting 40-70%, by weight, of the mixture.

5. A cogeneric mixture of conjugated polyoxyalkylene compounds containing in their structure oxypropylene groups, hydrophilic oxyalkylene groups having an oxygen/carbon atom ratio of at least 0.5 and an organic radical derived from an organic compound containing a plurality of reactive hydrogen atoms; the compounds being characterized in that all of the oxypropylene groups are present in polyoxypropylene chains that are attached to the organic radical at the site of a reactive hydrogen atom thereby constituting a polyoxypropylene polymer; the hydrophilic oxyalkylene groups being attached to the polyoxypropylene polymer in polyoxyalkylene chains; the average molecular weight of the polyoxypropylene polymers in the mixture being at least 900, as determined by hydroxyl number, and the hydrophilic oxyalkylene groups present constituting 20-90%, by weight, of the mixture.

6. A cogeneric mixture of conjugated polyoxy-alkylene compounds containing in their structure oxypropylene groups, hydrophilic oxyalkylene groups having an oxygen/carbon atom ratio of at least 0.5 and an organic radical derived from an organic compound containing a plurality of reactive hydrogen atoms; the compounds being characterized in that all of the oxypropylene groups are present in polyoxypropylene chains that are attached to the organic radical at the site of a reactive hydrogen atom thereby constituting a polyoxypropylene polymer; the hydrophilic oxyalkylene groups being attached to the polyoxypropylene polymer in polyoxy-alkylene chains; the average molecular weight of the polyoxypropylene polymers in the mixture being at least 900, as determined by hydroxyl number, and the hydrophilic oxyalkylene groups present constituting 40-70%, by weight, of the mixture.

7. A cogeneric mixture of conjugated polyoxyalkylene compounds containing in their structure oxypropylene groups, hydrophilic oxyalkylene groups having an oxygen/carbon atom ratio of at least 0.5 and an organic radical derived from an organic compound containing a plurality of reactive hydrogen atoms; the compounds being characterized in that all of the oxypropylene groups are present in polyoxypropylene chains that are attached to the organic radical at the site of a reactive hydrogen atom thereby constituting a polyoxypropylene polymer; the hydrophilic oxyalkylene groups being attached to the polyoxypropylene polymer in polyoxyalkylene chains; the average molecular weight of the polyoxypropylene polymers in the mixture being at least 2000, as determined by hydroxyl number, and the hydrophilic oxyalkylene groups present constituting 20-90%, by weight, of the mixture.

8. A cogenetic mixture of conjugated polyoxyalkylene compounds containing in their structure oxypropylene groups, hydrophilic oxyalkylene groups having an oxygen/carbon atom ratio of

16

at least 0.5 and an organic radical derived from an organic compound containing a plurality of reactive hydrogen atoms; the compounds being characterized in that all of the oxypropylene groups are present in polyoxypropylene chains that are attached to the organic radical at the site of a reactive hydrogen atom thereby constituting a polyoxypropylene polymer; the hydrophilic oxyalkylene groups being attached to the 10 polyoxypropylene polymer in polyoxyalkylene chains; the average molecular weight of the polyoxypropylene polymers in the mixture being at least 2000, as determined by hydroxyl number, and the hydrophilic oxyalkylene groups 15 present constituting 40-70%, by weight, of the mixture.

9. A cogeneric mixture of conjugated polyoxypropylene-polyoxyethylene compounds containing in their structure oxypropylene groups, oxyethylene groups and an organic radical derived from an organic compound containing a plurality of reactive hydrogen atoms and having a detergency factor of less than 100; the compounds being characterized in that all of the oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 900, as determined by hydroxyl number, and the oxyethylene groups present constituting 20-90%, by weight, of the mixture; said compounds having a carbon soil removal value of at least 100.

40 10. A cogeneric mixture of conjugated polyoxypropylene-polyoxyethylene compounds containing in their structure oxypropylene groups, oxyethylene groups and an organic radical derived from an organic compound containing a plurality of reactive hydrogen atoms and having a detergency factor of less than 100; the compounds being characterized in that all of the 45 oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 900, as determined by hydroxyl number, and the oxyethylene groups present constituting 50 40-70%, by weight, of the mixture; said compounds having a carbon soil removal value of at least 100.

60 11. A cogeneric mixture of conjugated polyoxypropylene-polyoxyethylene compounds containing in their structure oxypropylene groups, oxyethylene groups and an organic radical derived from an organic compound containing a plurality of reactive hydrogen atoms and having a detergency factor of less than 100; the compounds being characterized in that all of the oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 65 2000, as determined by hydroxyl number, and the

oxyethylene groups present constituting 20-90%, by weight, of the mixture; said compounds having a carbon soil removal value of at least 100.

12. A cogeneric mixture of conjugated polyoxypropylene-polyoxyethylene compounds containing in their structure oxypropylene groups, oxyethylene groups and an organic radical derived from an organic compound containing a plurality of reactive hydrogen atoms and having a detergency factor of less than 100; the compounds being characterized in that all of the oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 2000, as determined by hydroxyl number, and the oxyethylene groups present constituting 40-70%, by weight, of the mixture; said compounds having a carbon soil removal value of at least 100.

13. A cogeneric mixture of conjugated polyoxypropylene-polyoxyethylene compounds containing in their structure oxypropylene groups, oxyethylene groups and an organic radical derived from an organic compound containing a plurality of reactive hydrogen atoms, said compound having a molecular weight of less than 200, the reactive hydrogen atoms of said organic compound being members of functional groups containing an element selected from the group consisting of oxygen, sulfur and nitrogen; the compounds being characterized in that all of the oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 900, as determined by hydroxyl number, and the oxyethylene groups present constituting 20-90%, by weight, of the mixture; said compounds having a carbon soil removal value of at least 100.

14. A cogeneric mixture of conjugated polyoxypropylene-polyoxyethylene compounds containing in their structure oxypropylene groups, oxyethylene groups and an organic radical derived from a polyhydric alcohol having a molecular weight of less than 200; the compounds being characterized in that all of the oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 900, as determined by hydroxyl number, and the oxyethylene groups present constituting 20-90%, by weight, of the mixture.

15. A cogeneric mixture of conjugated poly-

oxypropylene-polyoxyethylene compounds containing in their structure oxypropylene groups, oxyethylene groups and an organic radical derived from a carboxylic acid amide having a molecular weight of less than 200; the compounds being characterized in that all of the oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 900, as determined by hydroxyl number, and the oxyethylene groups present constituting 20-90%, by weight, of the mixture.

16. A cogeneric mixture of conjugated polyoxypropylene-polyoxyethylene compounds containing in their structure oxypropylene groups, oxyethylene groups and an organic radical derived from an arylsulfonamide having a plurality of reactive hydrogen atoms and a molecular weight of less than 200; the compounds being characterized in that all of the oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 900, as determined by hydroxyl number, and the oxyethylene groups present constituting 20-90%, by weight, of the mixture.

17. A cogeneric mixture of conjugated polyoxypropylene-polyoxyethylene compounds containing in their structure oxypropylene groups, oxyethylene groups and an organic radical derived from a polybasic carboxylic acid having a molecular weight of less than 200; the compounds being characterized in that all of the oxypropylene groups are present in polyoxypropylene chains that are attached to the organic radical at the site of a reactive hydrogen atom thereby constituting a polyoxypropylene polymer; the oxyethylene groups being attached to the polyoxypropylene polymer in polyoxyethylene chains; the average molecular weight of the polyoxypropylene polymers in the mixture being at least 900, as determined by hydroxyl number, and the oxyethylene groups present constituting 20-90%, by weight, of the mixture.

18. Compounds having improved detergent properties, according to the formula:



where  $y$  equals at least 15; and  $(\text{C}_2\text{H}_4\text{O})_{x+z}$  equals 20-90%, of the total weight of the compound.

References Cited in the file of this patent

UNITED STATES PATENTS

| Number    | Name             | Date          |
|-----------|------------------|---------------|
| 2,549,439 | De Groote et al. | Apr. 17, 1951 |
| 2,552,529 | De Groote        | May 15, 1951  |